

## UNITED STATES PATENT OFFICE

2,112,275

## SAPONIFICATION OF CELLULOSE ESTERS

Henry Dreyfus, London, England

No Drawing. Application January 4, 1935, Serial No. 327. In Great Britain January 15, 1934

8 Claims. (Cl. 8—20)

This invention relates to improvements in the treatment of filaments, threads, yarns, fabrics and the like and is more particularly concerned with processes for the saponification of textile and other materials containing cellulose esters.

I have found that it is of advantage in the saponification of materials of the type referred to above, particularly when using strongly alkaline saponifying agents such for example as caustic soda, to have present a small quantity of a salt of the saponifying agent with an aromatic substance of weakly acid reaction. Thus for example it is of advantage when saponifying such materials by means of caustic soda to have present small quantities of the sodium salt of phenol, salicylic acid, benzoic acid or other phenol or aromatic carboxylic acid. In the presence of small quantities of such substances saponification can be carried out rapidly without damaging the materials or undesirably reducing their tenacity or extensibility.

The term "phenols" is intended to include not only phenol itself and its homologues such as cresol, but in addition di- and polyhydric phenols for example resorcinol, pyrocatechin, hydroquinone, phloroglucinol, pyrogallol and the like and substitution products of the phenolic bodies and especially carboxy substitution products such as salicylic acid. The carboxy substitution products appear to give better results qua the textile properties of the saponified materials than the simple phenols.

The saponifying agent preferably comprises an aqueous solution of caustic soda or caustic potash. The solution may be of relatively low concentration, for instance from 1 or 2% or even less to 3 or 4%, or of considerably higher concentration, for instance 5-10 or 15%. The bath may be at atmospheric temperature or below atmospheric but for rapid saponification somewhat higher temperatures are preferable and the bath may even be maintained at a temperature just short of the boiling point.

The phenol or its equivalent is preferably dissolved in the saponifying medium, although other suitable methods of application are not excluded. The phenol or the like should be present in small quantity, for example in a concentration of the order of 0.2-0.5% up to 1% based on the total saponifying medium.

The saponifying medium may be applied in any suitable manner. The invention includes simple treatments of hanks or other packages in a bath, the treatment of travelling filaments in which case the saponifying conditions are preferably

adjusted so as to produce rapid saponification, or the type of process in which the material undergoing treatment is first impregnated with the appropriate amount of saponifying agent, for example in a bath or in a padding mangle or like impregnating machine and is subsequently heated, for example by passage over heated drums or other heated surfaces to effect a rapid saponification. Similarly spinning box cakes, yarn wound on perforated bobbins or other foraminous support may have the saponifying medium circulated through them. Travelling materials are preferably treated in warp formation, that is to say a large number of yarns, threads or the like are aligned and carried together through the saponifying treatment with the aid of rollers or other driving means operating upon the sheet of yarns as a whole. In this way great uniformity of treatment can be obtained with resultant uniformity in the properties, and particularly in the dyeing properties of the materials treated.

The invention includes both partial and complete saponification. For example in the case of treating cellulose acetate materials the saponification may be such as to remove 10-20 or 30% of the original acidyl content of the ester and may be for the purpose of increasing the safe ironing point of the materials or generally increasing their resistance to heat treatments and/or for the purpose of conferring thereon an affinity for cotton colours, or may be such as to remove a much greater proportion of the original acidyl content such as 50-70 or 75%, or to produce complete saponification.

As indicated above the phenol or equivalent substance or sodium phenate or other reaction product of the substance with the saponifying medium is preferably incorporated directly in an aqueous solution of caustic alkali or other alkaline substance so as to make up the saponifying medium. However, the yarns, threads, fabrics or other materials may if desired be impregnated with the phenol or phenate prior to contact with the saponifying medium. In order to obtain a good impregnation the phenolic substance may be applied in the free state rather than in the form of a phenate. In such a preliminary impregnation care should be taken that the concentration of the phenol in the pretreatment bath does not produce incipient solution of the cellulose ester unless at the same time mutual adherence of filaments to make for example a monofil or ribbon is desired.

The saponifying medium may contain in addition to the saponifying agent and the phenolic

substance any other desired constituents, as for example swelling agents for the cellulose ester under treatment. For example, when cellulose acetate materials are treated the saponifying medium may contain ethylene methylene ether, di-oxane or acetone.

The following example illustrates the invention:—

*Example*

- 10 Cellulose acetate yarn is drawn from a creel in warp formation through a saponifying bath, through a washing bath which removes residual alkali carried over from the saponifying bath, and over a series of steam heated drying rolls to suitable collecting means. The saponifying bath contains an aqueous solution of caustic soda of relatively low concentration, in which is dissolved a small quantity of sodium phenate.
- 15 Instead of phenol, other like acting substances may be employed, for example resorcinol, phloroglucinol or salicylic acid.

The process of the invention is particularly applicable to the treatment of cellulose acetate materials but may be applied to other organic esters of cellulose, for example cellulose formate, propionate, butyrate, oxy-ethyl acetate and the like. The tensile strength of the resulting products may be improved by stretching the materials, preferably before the saponifying treatment and either during or after the spinning of the materials, for example stretching them under the action of a softening agent, for instance the solvents mentioned above, to 200 to 300 or even 500% or more of their original length. Furthermore, it is advantageous to employ cellulose esters of high viscosity characteristics, for example, in the case of cellulose acetate, products having a viscosity of above 40 and preferably more than 50 to 100 or even 200 or more as measured by a comparison of the viscosity of a 6% solution of the cellulose acetate in acetone against that of glycerine taken as a standard of 100.

What I claim and desire to secure by Letters Patent is:—

1. Process of saponifying filaments, threads, ribbons and like materials composed substantially of organic esters of cellulose comprising treating the same with a bath containing an alkaline saponifying agent and small quantities of a salt

of said agent with an aromatic substance of weakly acid reaction selected from the group consisting of phenols and carboxylic acids.

2. Process of saponifying filaments, threads, ribbons and like materials composed substantially of organic esters of cellulose comprising treating the same in an aqueous caustic alkali bath containing small quantities of the salt of said alkali with a phenol.

3. Process of saponifying filaments, threads, ribbons and like materials composed substantially of organic esters of cellulose comprising treating the same in an aqueous caustic alkali bath containing small quantities of the salt of said alkali with an aromatic carboxylic acid.

4. Process for the treatment of filaments, threads, ribbons and like materials composed substantially of organic esters of cellulose which comprises subjecting the materials to substantially complete saponification by treatment with a bath containing caustic alkali and small quantities of a salt of said alkali with an aromatic substance of weakly acid reaction selected from the group consisting of phenols and carboxylic acids.

5. Process of saponifying filaments, threads, ribbons and like materials composed substantially of cellulose acetate comprising treating the same with a bath containing aqueous caustic alkali and small quantities of a salt of said alkali with ordinary phenol.

6. Process of saponifying filaments, threads, ribbons and like materials composed substantially of cellulose acetate comprising treating the same with a bath containing aqueous caustic alkali and small quantities of a salt of said alkali with resorcinol.

7. Process of saponifying filaments, threads, ribbons and like materials composed substantially of cellulose acetate comprising treating the same with a bath containing aqueous caustic alkali and small quantities of a salt of said alkali with a phenolic carboxylic acid.

8. Process of saponifying filaments, threads, ribbons and like materials composed substantially of cellulose acetate comprising treating the same with a bath containing aqueous caustic alkali and small quantities of a salt of said alkali with salicylic acid.

HENRY DREYFUS.